

U. S. PATENT OFFICE

TELEGRAPHIC ADDRESS

Feb. 1, 1927.

1,615,957

E. E. SCHUMACHER

SINTERING REFRACTORY METALS

Filed Oct. 2, 1923



Inventor:  
Earle E. Schumacher,  
by Jas C. Launer Atty

## UNITED STATES PATENT OFFICE.

EARLE E. SCHUMACHER, OF EAST ORANGE, NEW JERSEY, ASSIGNOR TO WESTERN ELECTRIC COMPANY, INCORPORATED, OF NEW YORK, N. Y., A CORPORATION OF NEW YORK.

## SINTERING REFRACRY METALS.

Application filed October 2, 1923. Serial No. 666,142.

This invention relates to the sintering of metals and has for its object the production of coherent bodies of highly refractory metals.

5 This object is attained by supporting in a vacuum a mass of finely divided refractory metal and passing a relatively high electric current through the mass to heat it to a sufficiently high temperature to sinter it.

10 Referring now to the drawings, this single figure thereof discloses an apparatus for treating the metal.

A glass vessel 10 is provided with a neck 11 and a conduit 12 which is adapted to 15 lead to a vacuum pump, (not shown). A tubular extension 13 protrudes from the vessel at a point opposite the neck 11 and has sealed at its end a copper disk 14 according to the method disclosed in the patent to 20 W. G. Houskeeper 1,293,441 of February 4, 1919. A leading-in conductor 15 passes through the disk 14 and is soldered or otherwise connected to the disk and projects up through the portion 13.

25 A tubular ground glass stopper 16 is provided to fit in the neck 11 and close the vessel. A copper disk 17 is sealed to the outer end of the stopper 16 according to the method disclosed in the aforementioned

30 Housekeeper patent and is provided with a leading-in conductor 18 which extends into the interior of the vessel 10. A tubular clamp 19 is threaded on to the end of the conductor 18 and is provided with a nut 20

25 for tightening the clamp. Held by the clamp is a body 21 of finely divided refractory metal compressed into a bar or rod. In the protruding portion 13 is provided a supply of mercury 22 into which dips a 40 metal sleeve 23 carried by the rod 21. The conductor 15 projects up into the sleeve 23.

With a rod 21 supported in the manner shown, the conduit 12 is connected to an exhaust pump and the gas exhausted from 45 the vessel 10. The leading-in conductors 15

and 18 are connected with a suitable source of electrical energy and current passed through the rod 21 to heat it to a sufficiently high temperature to sinter it.

This apparatus and method obviate the 50 necessity of using hydrogen during the sintering process as it is possible to remove all injurious gases from the presence of the rod, and also permit the observation of the metal during the sintering process. 55

It is, of course, understood that various modifications may be made in this apparatus without departing in any way from the spirit of the invention, as set forth in the appended claims. 60

The invention claimed is:

1. Apparatus for sintering bars of compressed metallic powder comprising an evacuable vessel, vacuum tight conductors for leading current into and out of said vessel, 65 clamp fastenings for leading current into and out of said bar, means for attaching one of said conductors to one of said fastenings, a pool of mercury so disposed as to electrically connect the other said fastening 70 to the other said conductor so that said bar may contract or expand freely.

2. In combination, a vessel having a neck and a tubular projecting portion, a metal disk sealed in the end of said tubular portion, an electrical conductor passing through said disk, a tubular stopper for said neck, a metal disk sealed in said stopper, a leading-in conductor passing through said disk, a clamp at the end of said conductor, a body 80 of metal supported by said clamp, a supply of mercury in said tubular portion, and a tubular metallic member attached to the end of said body of metal and extending into said mercury. 85

In witness whereof, I hereunto subscribe my name this 25th day of September A. D., 1923.

EARLE E. SCHUMACHER.